

Feb. 9, 1960

E. J. GRISET, JR., ET AL

2,924,000

## BULKING YARN

Filed Jan. 26, 1955



## INVENTORS

*Ernest J. Griset, Jr.<sup>a</sup>  
James A. McIntosh*

Met R. Poston

**ATTORNEY**

1

2,924,000

## BULKING YARN

Ernest J. Griset, Jr., Asheville, and James A. McIntosh, West Asheville, N.C., assignors, by mesne assignments, to E. I. du Pont de Nemours and Company, Wilmington, Del., a corporation of Delaware

Application January 26, 1955, Serial No. 484,218

4 Claims. (Cl. 28—1)

This invention relates to the production of continuous filament yarn characterized by the presence of tight curls or loops of small diameter, and, if desired, localized areas of increased denier.

In commonly owned application Serial No. 460,166, filed October 4, 1954, now U.S. Patent Number 2,874,445, there is disclosed a method and apparatus for bulking continuous filament yarn. In that application there is disclosed a nozzle for projecting an air jet into which the yarn to be bulked is led. This air jet impinges against a baffle and it has been found that the spacial relation between the end of the nozzle and the baffle is an important factor in controlling the diameter of the loops which are formed. In general the smaller the distance between the nozzle and baffle the smaller will be the diameter of the loops produced. However, it has been found that the production of very small diameter loops is fraught with great difficulty which is not overcome even by locating the baffle very close to the nozzle.

It is an object of this invention to overcome the foregoing difficulty and to provide a method and apparatus for the production of bulky yarn characterized by curls or loops of extremely small diameter of the order of the diameter of the thread undergoing bulking.

Other objects and advantages of this invention will be apparent from a consideration of the following description of several embodiments thereof in conjunction with the annexed drawings wherein:

Figure 1 is a schematic view in elevation showing a yarn or thread supply package, a bulking mechanism incorporating the improvements of the present invention and the package take-up apparatus;

Figure 2 is a view in longitudinal section of a nozzle assembly showing the spiral wire of the present invention in operative position;

Figure 3 is a view in transverse section taken on the line 3—3 of Figure 2;

Figure 4 is a detailed view to an enlarged scale of a preferred jet tube according to the present invention, the illustrated tube being divorced from the nozzle such as is shown in Figure 2; and

Figure 5 is a view similar to Figure 4 but showing a modified type of jet tube according to the present invention.

Referring now in greater detail to the drawings, the numeral 10 designates a supply package containing yarn to be bulked. This yarn is led through guides 11, 12 and 13 to and around a large sheave or pulley 14 of a two-step coaxial pulley system including also a small sheave or pulley 15. The pulleys 14 and 15 are fixed together but mounted for free rotation on a shaft 16 which is supported from a bracket 17, which is, in turn, fastened to a fitting 18. The fitting 18 has a threaded end 19 which is connected to coupling 20.

The yarn leaving the underside of the large pulley or sheave 14 runs to and over a guide 21 into a notch 22 in a jet tube or conduit 23 to be acted upon by a stream of air under pressure supplied from coupling 20. After

2

leaving the conduit 23, the yarn is subjected to the influence of air impinging against a baffle plate 24 and is then led over various guides to a tension controlling feeler arm 25. As is described in application Serial No. 460,166, the feeler arm 25 adjusts a brake bearing on the sheaves 14 and 15 inversely as a function of the tension of the yarn running from the feeler arm 25 to the take-up spool 26. A spring 27 does the braking and, if less tension is needed, arm 25 functions to relieve some of the bias imposed on the brake by the spring 27.

If now reference is made to Figures 2, 3 and 4, it can be seen that tube 23 is provided with an internal spiral wire 28 which has enough radial bias to retain itself in position by friction. When yarn is bulked by using the apparatus of Figure 1 with the improvement shown in Figures 2, 3 and 4 and with the baffle 24 about  $\frac{1}{16}$  inch from the discharge end of the tube 23 excellent bulky yarn is produced, the yarn being characterized by very small loops or curls. It appears that the turbulence created by the swirling of the air caused by the spiral wire 28 is probably the cause of the small diameter loops. Best results have been observed when the air is caused to revolve in the same direction as the twist in the yarn although this is not critical. Results are also good when the yarn is withdrawn from the baffle area opposite to the direction of the air, i.e., opposite to the direction of the arrow of Figure 2. This too is preferred but not critical.

Although excellent results have been achieved by inserting a spiral wire in the tube of the nozzle assembly as shown in Figure 4, it is also possible to achieve the same effect by cutting or milling lands or grooves in the bore of the tube much as in the rifling of fire arms. An example of this is shown in Figure 5 where spiral lands 29 have been machined inside a tube 30 otherwise corresponding in structure and function to tube 23. The width of the lands 29 or intermediate grooves 31 can be varied to suit different conditions of operation. Likewise the helix angle can be varied although a helix angle generally corresponding to the yarn twist is desirable.

The portion of the length of the bore of the tube that is provided with a spiral wire or with lands and grooves is a matter of how much is needed to baffle the air into a spiral path. Equally satisfactory results have been obtained when the spiral wire occupies substantially the full length of tube 23 or when it occupies only the small diameter portion thereof. The invention will be further illustrated by the following examples:

## EXAMPLE I

50 300/75 acetate yarn having 5 t.p.i. of Z twist was passed through a bulking device as shown in Figure 1. The diameter of the small pulley was 0.9375 inch, and the diameter of the large pulley was 1.125 inches. The nozzle section of the jet was  $\frac{1}{4}$  inch long with an internal diameter of 0.047 inch, and the venturi section was 1 inch long with an internal diameter of 0.067 inch. A spiral wire 0.020 inch in diameter and containing 4 t.p.i. of Z twist was inserted in the nozzle and the venturi section of the jet as shown in Figure 4. The baffle 60 at the exit end of the jet formed an angle of 100° with respect to the axis of the jet. The distance from the jet to the baffle at the closest point was  $\frac{1}{64}$  inch. The air pressure was adjusted to a consumption of 2 c.f.m., and the yarn was collected on a tube winder take-up 65 without imparting any additional twist. The take-up speed was 54 yards per minute, and the take-up tension was 35 grams.

The yarn was bulked with the foregoing apparatus, both with and without the spiral wire. The average diameter of the main yarn body, exclusive of loops or curls, was approximately 0.3 mm. The loops or curls that were produced in the bulked yarn were measured and com-

pared with the diameter of the main yarn body. When using the spiral in the jet, about 75% of the loops were 0.3 mm. or less. Rarely did the larger loops exceed 0.6 mm. When the spiral was not used in the jet, more than 50% of the loops were larger than 0.3 mm; in some cases they were as large as 1 mm.

Table II gives the increase in denier, with and without the spiral present in the jet:

Table I

|                     | Unbulked | Bulked | Percent Denier Increase |
|---------------------|----------|--------|-------------------------|
| Without spiral..... | 302.9    | 327.8  | 8.2                     |
| With spiral.....    | 302.9    | 332.6  | 9.8                     |

## EXAMPLE II

This example was run on the same apparatus as described in Example I with the following changes: The yarn used was 150/40 viscose rayon containing 5.5 t.p.i. of S twist; a spiral wire containing 4 t.p.i. S twist was used; the air consumption was adjusted to 2.5 c.f.m.

The diameter of the main yarn body was approximately 0.25 mm. When the spiral wire was used, about 10% of the loops were larger than 0.25 mm. When the spiral wire was not used, about 30% of the loops were larger than 0.25 mm.

Data on the change in denier, with and without the spiral wire, is given in Table II.

Table II

|                     | Unbulked | Bulked | Percent Denier Increase |
|---------------------|----------|--------|-------------------------|
| Without spiral..... | 150.9    | 161.6  | 7.1                     |
| With spiral.....    | 150.9    | 164.5  | 9.0                     |

What is claimed is:

1. The method of bulking yarn that comprises passing a stream of high velocity gas from a jet into a tubular passageway disposed in axial alignment with said jet, imparting a whirling effect to said stream of gas by spiral defining means disposed in said passageway, continuously passing a multifilament yarn into an opening communicating with said passageway and axially through said spiral defining means, subjecting said yarn to the action of the whirling gas stream while it passes axially through said spiral defining means, and abruptly changing the direction of yarn travel.

2. Apparatus for bulking yarn comprising a jet means in axial alignment with a tubular passageway discharging into the atmosphere, means to supply gas under high pressure to said jet means, means to continuously supply a yarn to an opening communicating with said tubular passageway, spiral defining means within said passageway to cause said gas to flow in contact with said yarn while said yarn is passed axially through said spiral defining means, said opening being disposed intermediate said jet means and the end of said tubular passageway discharging into the atmosphere, and means for changing the direction of yarn travel at the exit end of the tubular passageway.

3. Apparatus for bulking yarn comprising a jet means in axial alignment with a tubular passageway discharging into the atmosphere, means to supply gas under high pressure to said jet means, means to continuously supply a yarn to an opening communicating with said tubular passageway, a spiral wire within said passageway to cause said gas to flow in a spiral path in contact with said yarn while said yarn is passed axially through said spiral wire, said opening being disposed intermediate said jet means and the end of said tubular passageway discharging into the atmosphere, and means for changing the direction of yarn travel at the exit end of the tubular passageway.

4. Apparatus for bulking yarn comprising a jet means in axial alignment with a tubular passageway discharging into the atmosphere, means to supply a gas under high pressure to said jet means, means to continuously supply a yarn to an opening communicating with said tubular passageway, an integral spiral land within said passageway to cause said gas to flow in a spiral path in contact with said yarn while said yarn is passed axially through said spiral land, said opening being disposed intermediate said jet means and the end of said tubular passageway discharging into the atmosphere, and means for changing the direction of yarn travel at the exit end of the tubular passageway.

## References Cited in the file of this patent

## UNITED STATES PATENTS

|           |                    |               |
|-----------|--------------------|---------------|
| 2,100,588 | Claus              | Nov. 30, 1937 |
| 2,125,230 | Hofmann            | July 26, 1938 |
| 2,379,824 | Mummery            | July 3, 1945  |
| 2,638,146 | Rounseville et al. | May 12, 1953  |
| 2,681,729 | Griset             | June 22, 1954 |
| 2,783,609 | Breen              | Mar. 5, 1957  |

## FOREIGN PATENTS

|         |         |               |
|---------|---------|---------------|
| 495,767 | Germany | Apr. 11, 1930 |
|---------|---------|---------------|